

3,355,294  
**PHOTOCROMIC COMPOSITIONS CONTAINING  
 BLEACHING RATE ACCELERATORS**  
 Sydney Arthur Giddings, New Canaan, Conn., assignor to  
 American Cyanamid Company, Stamford, Conn., a corpora-  
 tion of Maine  
 No Drawing. Filed Dec. 9, 1964, Ser. No. 417,234  
 14 Claims. (Cl. 96—90)

## ABSTRACT OF THE DISCLOSURE

Photochromic compositions comprising an oxygen-containing polymer, certain metal compounds and various metal salts which, in solution, have an oxidation potential of from about —.30 to about —1.65 are disclosed.

This invention relates to novel compositions of matter. More particularly, this invention relates to novel compositions of matter comprising an oxygen-containing polymeric material, a transition metal compound and a bleaching rate increasing additive. Still more particularly, this invention relates to novel compositions of matter comprising (1) a polymeric material, (2) a solvent therefor, (3) a transition metal compound having the formula



wherein M is a transition metal, X is a halide, R is an alkyl radical having from 1 to 12 carbon atoms, inclusive, an aryl radical having from 6-10 carbon atoms, inclusive, or a



radical,  $\text{R}^1$  is an alkyl radical having from 1-12 carbon atoms, inclusive, or an aryl radical having from 6-10 carbon atoms, inclusive,  $m$  and  $p$  are whole, positive integers of from 0-6, inclusive, and  $n$  is a whole, positive integer of from 0-2, inclusive, the total of  $2n+m+p$  being equal to the valence of the metal M, at least one of  $m$  and  $p$  being an integer of at least 1, and at least one of said polymeric material and said solvent containing oxygen and (4) a bleaching rate increasing additive.

I have discovered that the bleaching rate of certain photochromic compositions composed of plastic materials and certain transition metal compounds can be materially increased by the addition of a specific group of additives thereto. The additives have been found to increase the bleaching rate, i.e., the rate of color change of the composition which has been irradiated, from its color caused by the irradiation back to its original color, as much as 10-50% over the bleaching rate of the untreated composition. The compositions of the instant invention still function photochromically in the form of various articles, such as sheets, films and the like when subjected to ultraviolet light.

The use of photochromic materials as active ingredients in such applications as data storage devices, absorbers for incident, high-intensity radiation, photochemical printing, variable transmission devices and the like is well-known in the art. Compositions of matter which function photochromically and which may be utilized for these purposes are the subject matter of various patents. I have now found that compositions of matter composed of a polymeric material, a solvent and a transition metal compound can be further enhanced so that they may be utilized for additional applications wherein rapid bleaching rates are essential, by the addition of a group of various bleaching rate increasing additives thereto.

It is therefore an object of the present invention to provide novel compositions of matter.

It is a further object of the present invention to provide novel compositions of matter comprising a polymeric material, a transition metal compound and a bleaching rate increasing additive.

It is a further object of the present invention to provide compositions of matter which are composed of a polymeric, resinous material, a solvent therefor, at least one of which contains oxygen, a transition metal compound represented by Formula I, above, and a bleaching rate increasing additive, which compositions of matter are photochromic.

These and other objects of the present invention will become more apparent to those skilled in the art upon reading the more detailed description set forth hereinbelow.

## Photochromism

20 Molecules or complexes which undergo reversible photo-induced color changes are termed photochromic systems. That is to say, in the absence of activating radiation, the system has a single stable electronic configuration with a characteristic absorption spectrum. When the 25 system is contacted with ultraviolet irradiation, the absorption spectrum for the system changes drastically, but when the irradiation source is removed, the system reverts to its original state.

Photochromism has been observed in inorganic and 30 organic compounds both in solution and solid state. Although the exact mechanism of color change varies markedly in each individual system, there are two processes which account for most types of photochromic phenomena. The first process is the transformation of 35 excited state electronic energy into vibrational and torsional twisting modes of the molecule. Usually, systems observed to be photochromic have very efficient routes for internal transformation of absorbed energy and are generally never fluorescent or phosphorescent. Internal 40 transformation often takes place very rapidly. That is to say, the primary process in the photo-production of a colored species often occurs in about a millimicrosecond. However, optical observation of the colored species normally takes considerably longer than this because of the 45 very small amounts of colored material produced per unit time and the depletion of the color by the competing reverse reaction.

The second fundamental photo-electronic mechanism generally considered as producing photochromism is charge transfer. Most charge transfer phenomena in organic molecules are rapidly reversible and therefore produce no colored intermediate. However, in inorganic crystals, charge transfer absorption usually leads to a colored 50 state in which the donor-acceptor crystals have been oxidized and reduced.

There are three major factors which govern the behavior of a photochromic system.

A. *Absorption of incident radiation.*—According to the 55 quantum theory, each absorbed quantum creates one activated molecule and only absorbed radiation can produce a chemical change. Variables which control the number of photons absorbed include the concentration and extinction coefficient of the photochrome, the cell length, the screening coefficients of other components of the system, and the wavelengths of the incident radiation.

B. *Quantum yield.*—All excited molecules will not undergo transformation to the colored form, so that the quantum yields will generally be less than unity. Various deactivating processes which compete for the excited molecules include fluorescence, phosphorescence, permanent 60 chemical change and the thermal release.

C. *The reverse reaction.*—In both the forward and reverse reactions, the concentration of the colored form is dependent on the intensity of the radiation, the kinetics of the reverse reactions, and temperature and solvent sensitivity of the reactions. The kinetics for the reverse reaction will normally be controlling, however, some reverse reactions are thermally sensitive and are accelerated by irradiation.

The terms "photochromic composition" or "photochromic material," and the like, as used in the instant disclosure, mean compositions or materials, etc., which change their transmission or reflectance upon being subjected to ultraviolet or visible irradiation and subsequently revert to their original state upon subjection thereof to a different wavelength of radiation or removal of the initial ultraviolet source.

The ability of various materials to change color and to then revert back to their original color is not a new phenomena. In fact, such compounds have been widely used in various ways, as described above. Generally these compounds change their color when exposed to ordinary sunlight and revert back to their original color upon removal thereof from the rays of the sun. Various other materials, however, change color only when subjected to a certain degree of irradiation, and as such, sunlight will not effect them. High intensity radiation, such as 10-25 cal./cm.<sup>2</sup>/sec. or more is necessary in regard to these compounds, while sunlight (0.2 cal./cm.<sup>2</sup>/sec.) will affect the former.

#### *The compositions of matter*

As mentioned above, I have found that the bleaching rate of various compositions of matter composed of a polymeric material and a transition metal compound represented by Formula I, above, can be increased by blending a group of specific bleaching rate increasing additives therewith. I have further found that the presence of a solvent for the polymer in these compositions is a material advantage. The only critical requirement in regard to the components in the compositions of matter is that at least one of the polymer or the solvent, if present, must contain oxygen, either in combined or free form. That is to say, the compositions of the present invention are photochromic when formed into shaped articles only when the plastic component, the solvent component, or both, contain oxygen in some form, such as combined with the other elements of the component in question or in free form, i.e., as an added entity, e.g., an impurity or the like. Of course, when no solvent is employed in the compositions of matter, the polymeric component thereof must be the oxygen-containing portion before any photochromic phenomena can be observed.

Any thermoplastic resin can be used in the formation of our novel compositions of matter. That is to say, any polymeric material, synthetic or naturally occurring, which is thermoplastic in nature and which may be dissolved in a solvent or made molten, may be used herein. Evidence of the types of polymers useful in our invention can be obtained from the more detailed description thereof set forth immediately hereinbelow.

Examples of thermoplastic resinous or plastic materials which may be utilized in the preparation of the compositions of the present invention are the various esters of acrylic acid and methacrylic acid, e.g., those having the formula



wherein R<sup>2</sup> is hydrogen or a methyl radical and R<sup>3</sup> is an alkyl radical having from 1 to 6 carbon atoms, inclusive. Compounds which are represented by Formula II and consequently may be used singularly or in admixtures with one another, as monomers from which the polymers used in the present invention may be produced include methyl

acrylate, ethyl acrylate, n-propyl acrylate, isopropyl acrylate, n-butyl acrylate, isobutyl acrylate, t-butyl acrylate, n-amyl acrylate, isoamyl acrylate, t-amyl acrylate, hexyl acrylate, methyl methacrylate, ethyl methacrylate, n-propyl methacrylate, isopropyl methacrylate, n-butyl methacrylate, isobutyl methacrylate, t-butyl methacrylate, n-amyl methacrylate, isoamyl methacrylate, t-amyl methacrylate, hexyl methacrylate and the like.

Other polymers which may be employed are those produced from styrene monomers, e.g., those having the formula

(III)



wherein R<sup>4</sup> is hydrogen or a lower alkyl radical having 1 to 4 carbon atoms, inclusive, and R<sup>5</sup> is hydrogen, a lower alkyl radical having 1 to 4 carbon atoms, inclusive or a halogen radical. Suitable monomers represented by Formula III include styrene, methyl styrene, ethyl styrene, propyl styrene, o-, m-, or p-butyl styrene, o-, m-, or p-chloro styrene, o-, m-, or p-bromo styrene, o-, m-, or p-fluoro styrene o-, m-, or p-iodo styrene,  $\alpha$ -methyl styrene,  $\alpha$ -ethyl styrene,  $\alpha$ -butyl styrene,  $\alpha$ -methyl-o-, m- or p-methylstyrene,  $\alpha$ -methyl-o-, m- or p-ethyl styrene,  $\alpha$ -butyl-o-, m- or p-ethylstyrene,  $\alpha$ -ethyl-o-, m- or p-chlorostyrene,  $\alpha$ -propyl-o-, m- or p-iodostyrene and the like.

Further examples of polymers which may be utilized to produce the novel compositions of the present invention include polymers of acrylonitrile, polymers of acrylamide, polymers of vinyl halides such as poly(vinyl chloride); polymers of vinylidene halides such as poly(vinylidene chloride); polymers of vinyl carbonate, vinyl alcohol, vinyl acetate, vinyl butyral; polymers of various aldehydes, such as oxymethylene, acetaldehyde, crotonaldehyde; polymers of ethyleneoxide; cellulose polymers such as cellulose acetate butyrate, cellulose triacetate, and any other polymeric material with which the transition metal compound is compatible in the molten state and preferably which may be dissolved in an appropriate solvent.

Additionally, the monomers represented by Formulae II and III above, and which are disclosed hereinabove as useful for producing homopolymers can be copolymerized either singly or in a plurality (two, three, four or any desired number), the latter often being desirable in order to improve the compatibility and copolymerization characteristics of the mixture of monomers with themselves or various other copolymerizable monomers to obtain copolymers having the particular properties desired for the particular service application. Examples of such comonomers are the unsaturated alcohol esters, more particularly the allyl, methallyl, 1-chloroallyl, 2-chlorallyl, cinnamyl, vinyl, methvinyl, 1-phenylallyl, etc., esters of saturates aliphatic and aromatic monobasic and polybasic acids such, for instance, as acetic, propionic, butyric, valeric, caproic, oxalic, malonic, succinic, glutaric, adipic, pimelic, suberic, azelaic, sebacic benzoic phenylacetic, phthalic, terephthalic, benzoylphthalic, etc., acids; vinyl naphthalene, vinylcyclohexane, vinyl furane, vinyl pyridine, vinyl dibenzofuran, divinyl benzene, trivinyl benzene, allyl benzene, diallyl benzene, N-vinyl carbazole, unsaturated ethers, e.g., ethyl vinyl ether, diallyl ether, ethyl methallyl ether, etc.; unsaturated amides, for instance, N-allyl caprolactam, N-substituted acrylamides, e.g. N-methylol acrylamide, N-allyl acrylamide, N-methyl acrylamide, N-phenyl acrylamide, etc.; unsaturated ketones, e.g., methyl vinyl ketone, methyl allyl ketone, etc.; methylene malonic esters, e.g., methylene methyl malonate, etc.

Further examples of thermoplastic polymers useful in producing my novel compositions are thermoplastic polyesters such as those produced by reacting a saturated ali-

phatic diol with a non-polymerizable polycarboxylic acid to produce a polyester having an acid number not appreciably more than 75. Among the dihydric alcohols which may be employed are saturated aliphatic diols such as ethylene glycol, propylene glycol, butylene glycol, diethylene glycol, dipropylene glycol, triethylene glycol, tetraethylene glycol, butanediol-1,2, butanediol-1,3, butanediol-1,4, pentanediol-1,2, pentanediol-1,3, pentanediol-1,4, pentanediol-1,5, hexanediol-1,2, hexanediol-1,3, hexanediol-1,4, hexanediol-1,5, hexanediol-1,6, neopentyl glycol, and the like, as well as mixtures thereof. Among the polyols having more than two hydroxyl groups which may be employed in minor amounts, together with the above-mentioned diols, are saturated aliphatic polyols such as glycerol, trimethylol ethane, trimethylol propane, pentaerythritol, dipentaerythritol, arabitol, xylitol, dulcitol, adonitol, sorbitol, mannitol, and the like, as well as mixtures thereof.

Non-polymerizable polycarboxylic acids, i.e., acids which are saturated or which contain only benzenoid unsaturation, which may be used include oxalic, malonic, succinic, glutaric, adipic, pimelic, suberic, azelaic, sebacic, malic, tartaric, tricarballylic, citric, phthalic, isophthalic, terephthalic, cyclohexanedicarboxylic, endomethylene-tetrahydrophthalic, and the like, as well as mixtures thereof.

The esterification mixtures, from which the thermoplastic polyester resins employed in the practice of the present invention are prepared, are generally formulated so as to contain at least a stoichiometric balance between carbonyl and hydroxyl groups. Thus, where a diol and a dicarboxylic acid are employed, they are usually reacted at elevated temperatures and in an inert atmosphere, on at least a mole to mole basis. In common commercial practice, a small excess of polyol, usually in the range of from about 5% to about 15% excess, is employed. This is done primarily for economic reasons, i.e., to insure a rapid rate of esterification.

Further details pertaining to the preparation of polyester resins of the types employed in the practice of the present invention are disclosed in U.S. Patent No. 2,255,313 to Ellis, and in U.S. Patent Nos. 2,443,735 to 2,443,741, inclusive, to Kropa, and these patents are hereby incorporated into the present application by reference.

As further examples of polymeric materials which may be used to produce my novel compositions of matter are the polyamide resins, i.e., those produced from a dibasic acid and a polyamine. Polyamide resins of this type are well known in the art and are generally termed "nylon" resins. These nylon resins, as used in the instant specification, are long chain synthetic polymeric amides which have recurring amide groups as an integral part of the main polymer chain and which are capable of being formed into a filament in which the structural elements are oriented in the direction of the axes. Most common of these nylons or polyamides are obtained by condensation of a diamine with a dicarboxylic acid or by auto condensation of an amino acid. These polyamides have the structural formula

(IV)



$x$  and  $y$  being greater than one. Methods for the production of polyamides of this type are shown, for example, in the following patents: U.S. Patent Nos. 2,191,556; 2,293,760; 2,293,761; 2,327,116; 2,359,877; 2,377,985; 2,572,843, said patents hereby being incorporated herein by reference.

Additionally, I may utilize such polymeric materials as the polyurethanes. Any polyester based or polyether based polyurethane resin may be used in the present invention. Among the reactive organic polyfunctional polyols employed in preparing one class of polyurethane resins used in the practice of our invention by reaction with a suitable isocyanate compound are the polyalkylene

ether, thioether, and ether-thioether glycols represented by the general formula



wherein  $\text{R}^6$  represents the same or different alkylene radicals containing up to about 10 carbon atoms,  $\text{X}^1$  represents oxygen or sulfur, and  $z$  is an integer large enough so that the molecular weight of the polyalkylene ether, thioether, or ether-thioether glycol is at least about 500, e.g., from about 500 to about 10,000. The polyalkylene ether glycols included within this general formula, such as polyethylene glycols, polypropylene glycols, polybutylene glycols, polytetramethylene glycols, polyhexamethylene glycols, and the like, which are obtained, for example, by acid-catalyzed condensation of the corresponding monomeric glycols or by the condensation of lower alkylene oxides, such as ethylene oxide, propylene oxide, and the like, either with themselves or with glycols such as ethylene glycol, propylene glycol, and the like, are preferred.

Polyalkylenearylene ether, thioether and etherthioether glycols which also have molecular weights ranging from about 500 to about 10,000 but which differ from the above-described polyalkylene glycols in having arylene radicals, such as phenylene, naphthylene and anthrylene radicals, either unsubstituted or substituted, e.g., with alkyl or aryl groups, and the like, in place of some of the alkylene radicals of said polyalkylene glycols may also be employed. Polyalkylene-arylene glycols of the type ordinarily used for this purpose will usually contain at least one alkylene ether radical having a molecular weight of about 500 for each arylene radical present.

Essentially linear polyesters containing a plurality of isocyanate-reactive hydroxyl groups constitute another class of reactive organic polyfunctional polyols which may be employed in preparing polyurethane resins useful in the practice of the present invention. While the preparation of polyesters suitable for this purpose has been described in great detail in the prior art and forms no part of the present invention per se, it may be mentioned here by way of illustration that polyesters of this type may be prepared by the condensation of a polyhydric alcohol, with a polycarboxylic acid or anhydride in the same manner as set forth hereinabove in regard to the dissertation on applicable polyester resins which may be used herein, with the same examples of reactants applying in both instances.

The essentially linear polyesters commonly used in preparing polyurethane resins preferably have molecular weights ranging from about 750 to about 3000. In addition they will generally have relatively low acid numbers, e.g., acid numbers not appreciably in excess of about 60 and preferably as low as can be practicably obtained, e.g., 2 or less. Correspondingly, they will generally have relatively high hydroxyl numbers, e.g., from about 30 to about 700. When preparing these polyesters, an excess of polyol over polycarboxylic acid is generally used to insure that the resulting essentially linear polyester chains contain a sufficient amount of reactive hydroxyl groups.

The polyurethane resins useful as a component of my novel compositions may be prepared using a wide variety of organic polyisocyanates, among which there are included the aromatic diisocyanates, such as m-phenylene-diisocyanate, p-phenylenediisocyanate, 4-t-butyl-m-phenylenediisocyanate, 4-methoxy-m-phenylenediisocyanate, 4-phenoxy-m-phenylenediisocyanate, 4-chloro-m-phenylenediisocyanate, toluediisocyanates (either as a mixture of isomers, e.g., the commercially available mixture of 80% 2,4-toluediisocyanate and 20% 2,6-toluediisocyanate, or as the individual isomers themselves), m-xylylenediisocyanate, p-xylylenediisocyanate, cumene-2,4-diisocyanate, durenediisocyanate, 1,4-naphthylenediisocyanate, 1,5-naphthylenediisocyanate, 1,8-naphthylenediisocyanate, 2,6-naphthylenediisocyanate, 1,5-tetrahydro-naphthylenediisocyanate, p,p'-diphenyldiisocyanate, di-

phenylmethane-4,4'-diisocyanate, 2,4-diphenylenehexane-1,6-diisocyanate, "bitolylenediisocyanate" (3,3-dimethyl-4,4' - biphenylenediisocyanate), "dianisidinediisocyanate" (3,3'-dimethoxy-4,4'-biphenylenediisocyanate), and polymethylenepolyisocyanates represented by the general formula



wherein  $b$  represents an integer between 0 and about 5, and the like; aliphatic diisocyanates, such as methylene-diisocyanate, ethylenediisocyanate, the tri-, tetra-, penta-, hexa-, hepta-, oct-, non- and decamethylene- $\omega,\omega'$ -diisocyanates, 2 - chlorotrimethylene-diisocyanate, 2,3-dimethyltetramethylene-diisocyanate, and the like, and tri- and higher isocyanates, such as benzene - 1,3,5 - triisocyanate, toluene - 2,4,6-triisocyanate, diphenyl-2,4,4'-triisocyanate, triphenylmethane-4,4',4''-triisocyanate, and the like. Mixtures of two or more of such organic polyisocyanates may also be employed to prepare the polyurethane resins by reaction with the ethers and esters described above utilizing procedures well known to those skilled in the art, see for example, U.S. Patents 2,729,618, 3,016,364 and the like.

As mentioned above, the polymer component of my novel compositions may be used as a molten material or as a solution thereof in a solvent. While the use of a solvent is preferred, it is not critical. The actual solvent employed in each instance is not critical except for the fact that it is preferred that the solvent contain an oxygen atom, as specified above. Generally, any compound which is a solvent for the polymer may be employed for this purpose in a sufficient amount so as to dissolve the polymer employed, provided that at least the polymer or the solvent contains oxygen, as mentioned above.

Examples of solvents which may be utilized include dimethyl formamide, acetonitrile, methylene chloride, glyme ( $\text{CH}_3\text{OCH}_2\text{CH}_2\text{OCH}_2\text{CH}_2\text{OCH}_3$ ), diglyme



chloroform, ethyl acetate, methylene chloride, trioxane, dioxane, ethyl formate, ethylene dichloride, isopropyl acetate, methyl acetate, acetic acid, acetone, benzil, acetaldehyde, benzaldehyde, butyl acetate, cellosolve, cyclohexanol acetate, cyclohexanone, methylethylketone, toluol, gamma-valerolactone, methanol, ethanol, hexanol, nitrobenzene, nitropropane, trichloroethylene, aniline, diacetone alcohol, ethyl lactate, carbon tetrachloride, pyridine, toluol, xylol, ethylene glycol, water and the like.

Additionally, any specific polymer may be dissolved in one of its own constituents so as to form a solution thereof. That is to say, poly(methyl methacrylate), for example, can be utilized as a solution of the polymer in methyl methacrylate. Likewise, the other polymers disclosed hereinabove may also be used as solutions thereof in monomers from which they are produced.

Furthermore, mixtures of the above-mentioned solvents or other solvents which conform to the requirements set forth herein, may be used to solubilize the polymers. For example, methylene chloride and acetic acid in a 50/50 mixture may be used with poly(methyl methacrylate).

In many instances, the polymers, as a result of solvents used during production thereof, or the solvents, as a result of affinity or weak bonding reactions, may contain a minor trace amount of an impurity such as water and the like. In instances of this sort, no newly added solvent need be added to produce our novel compositions if the critical oxygen requirement mentioned above has been fulfilled. By the term "trace amounts" or "impurities" is meant amounts as minimal as 0.1% are tolerable and

generally sufficient to enable the production of a photochromic article.

Examples of transition metal compounds which may be utilized in producing the compositions of matter of the present invention and which are represented by Formula I, include titanium tetrachloride, titanium oxidizedichloride, zirconium tetrachloride, zirconium oxidizedichloride, tungsten hexachloride, tungsten oxidetetrachloride, tungsten dioxidedichloride, hafnium tetrachloride, hafnium oxidizedichloride, tantalum pentachloride, tantalum oxidetrichloride, tantalum dioxidedichloride, hafnium tetraiodide, hafnium pentabromide, tantalum oxidetribromide, tantalum tetrabromide, zirconium tetrabromide, zirconium tetrabromide, zirconium oxidizedim bromide, tungsten hexabromide, tungsten oxidetetrabromide, tungsten dioxidedibromide, hafnium tetrabromide, hafnium oxidizedibromide, tantalum pentabromide, tantalum oxidetribromide, tantalum dioxidedibromide, titanium tetraiodide, titanium oxidediiodide, zirconium tetraiodide, zirconium oxidediiodide, tungsten dioxidediiodide, tungsten oxidetetraiodide, hafnium pentaiodide, hafnium oxidetriiodide, tantalum dioxideiodide, titanium tetrafluoride, titanium oxidedifluoride, zirconium tetrafluoride, zirconium oxidedifluoride, tungsten hexafluoride, tungsten oxidetetrafluoride, tungsten dioxidedifluoride, hafnium tetrafluoride, hafnium oxidedifluoride, tantalum pentafluoride, tantalum oxidetri fluoride, tantalum dioxidesfluoride, chromium dioxide dichloride, chromium dioxide dimethoxide, vanadium oxide trichloride, vanadium oxide triiodide, vanadium dioxide bromide, vanadium dioxide methoxide, titanium tetramethoxide, titanium tetraethoxide, titanium tetraheptoxide, titanium tetradecoxide, titanium oxide dimethoxide, titanium dichloride dimethoxide, titanium trichloride ethoxide, titanium chloride trimethoxide, zirconium tetramethoxide, zirconium tetraphenoxy, zirconium tetra(p-tolyloxy), zirconium tetra(naphthoxide), zirconium oxide dimethoxide, zirconium oxide diphenoxide, zirconium dibromide diethoxide, zirconium trifluoride butoxide, zirconium iodide trimethoxide, hafnium tetraacetate, hafnium tetravalerate, hafnium tetralaurate, hafnium oxide diacetate, hafnium dibromide divalerate, hafnium trifluoride laurate, hafnium chloride triphenoxide, tantalum pentamethoxide, tantalum pentabenzooate, tantalum penta(p-toluate), tantalum penta(2-naphthoate), tantalum oxide tribenzoate, tantalum dioxide methoxide, tantalum dichloride triethoxide, tantalum tetrabromide acetate, tantalum bromide tetraphenoxy, tantalum trifluoride dimethoxide, tungsten hexamethoxide, tungsten oxide tetrabenzoate, tungsten dioxide diacetate, tungsten pentachloride methoxide, tungsten tetrabromide bis(p-toluate), tungsten triiodide tris(p-tolyloxy), tungsten dichloride tetravalerate, tungsten bromide penta(1-naphthoate) and the like. The amount of transition metal employed may range from 0.01% to 50.0%, by weight, based on the weight of the polymer, preferably 0.1% to 25.0%, by weight, same basis.

The transition metal compounds listed above are all well known in the art and may be produced by any equally well known procedure. Examples of applicable methods for the production thereof appear in at least one of the following articles. Razivaer et al., *Tetrahedron* 6, 159 (1959); Sandho et al., *Current Sci. (Ind.)* 29, 222 (1960); Rosenheim, *Ch. Nernst. Z. Anorg. Chem.* 214, 220 (1933); Bradley et al., *J. Chem. Soc.* 1634 (1953), and these references are hereby incorporated herein by reference.

The additives which increase the bleaching rate of the photochromic compositions and form the crux of the present invention are defined as metal salts which, in solution, have oxidation potentials of from about -0.30 to about -1.65. The preferred metal salts are those which are colorless since the use of such salts enables one to maintain the color, whether it be water-white or red, of the resin-solvent-transition metal compound compositions to which they are added. The salts which possess

color, however, may be utilized if the final color of the composition is not critical and is not exactly the same as that to which the compositions devoid of the additives will change when subjected to ultra-violet light.

The amount of metal salts necessary to increase the bleaching rate of the photochromic compositions should range from about 0.01 mol to about 5.0 mols, preferably from about 0.1 mol to about 2.0 mols, of the metal salts, per mol of the transition metal compound represented by Formula I, above.

As mentioned above, the metal compounds which may be added to the photochromic compositions to increase the bleaching rate thereof must have an oxidation potential, in solution, of -3.0 to -1.65, inclusive. Generally salts of iron, thallium, manganese, cerium, rhodium, iridium and the like fall within these limits with such anions as the halides, i.e., chlorides, bromides, fluorides, iodides, the sulfates, the nitrates, oxylates, acetates, propionates, benzoates and the like being exemplary. That is to say, any salt which is formed by any cation and any coanion and has an oxidation potential within the above mentioned range may be used in my invention. Examples of salts which may be used include ferric chloride; ferrous chloride; ferric bromide; ferrous bromide; ferrous fluoride; ferric fluoride; ferric iodide; ferrous iodide; ferric sulfate; ferrous sulfate; ferric nitrate; ferrous nitrate; ferric oxylate; ferrous oxylate; ferric acetate; ferrous acetate; ferric propionate; ferrous propionate; ferric benzoate; ferrous benzoate; sodium arsenate; potassium arsenate; thallium chloride, iodide, fluoride, bromide, sulfate, nitrate, oxylate, benzoate, acetate and propionate; manganese bromide, chloride, iodide, fluoride, acetate, propionate, oxylate, benzoate, sulfate and nitrate; ceric and cerous chloride; bromide, iodide, fluoride, sulfate, nitrate, oxylate, acetate, benzoate and propionate; rhodium chloride, bromide, iodide, fluoride, sulfate, nitrate, oxylate, acetate, benzoate and propionate; potassium iridium chloride, bromide, iodide, fluoride, sulfate, nitrate, oxylate, benzoate and propionate; cupric and cuprous chloride, bromide, iodide, fluoride, acetate, propionate, benzoate nitrate, sulfate and oxylate and the like.

The order of the addition of the components to form my novel compositions is not critical and, furthermore, any method of blending may be used. For example, the solvent may be added to the polymer and then the transition metal compound and metal salt additive may be added or, alternatively, the transition metal compound and solvent may be blended and the resultant solution may then be blended with the resin to produce a composition to which may then be added the metal salt additive and so forth. If the polymer is used in a molten state in the absence of a solvent, however, the transition metal compound may be added thereto as such or as a mixture with the metal salt additive. The components may then be thoroughly admixed by utilizing such means as a Waring Blender, a ball mill, a rubber mill or the like, the specific device utilized for the blending in each instance forming no part of the instant invention.

Additionally, it is within the scope of the instant invention to form the compositions of matter claimed herein by first blending the oxygen-containing polymer (or other polymer if an oxygen-containing solvent is used) and solvent with the transition metal compound and metal salt to form a substantially uniform blend, precipitating the blend into a non-solvent for the polymer, transition metal compound and metal salt and recovering the resultant precipitated photochromic composition. Such a procedure is disclosed and claimed in copending application, Ser. No. 399,087, filed Sept. 24, 1964, which application and any other application or patent referred to herein is hereby incorporated herein by reference.

A further method for incorporating the metal salts into the compositions of the present invention is to con-

tact an oxygen-containing monomer (or other monomer if an oxygen-containing solvent is used), solvent, transition metal compound and metal salt with a polymerization catalyst under polymerizing conditions. By utilizing the method, which is disclosed and claimed in copending application Ser. No. 399,101, filed Sept. 24, 1964, a polymeric composition is recovered which is photochromic and has an increased return rate.

The novel compositions of the instant invention may be cast into films from a solution of the solvent by drawing the composition down on a self-supporting substrate such as glass, metals, such as steel, tile and the like, a resinous material such as polyethyleneglycol terephthalate, paper, cellophane, marble, wood, leather, cloth and the like, or merely casting on any solid surface and removing the resultant film. The thin film which is deposited by casting in this method generally should range in thickness from about 0.1 mil to about 1000 mils, preferably 0.5 mil to about 125 mils, to produce an optimum photochromic effect.

The exact phenomena which occurs upon blending the components of the compositions claimed herein is not completely understood. It is known however, that the compositions are not photochromic unless at least the thermoplastic resin or the solvent, or both, contain oxygen, in free or combined form, and until the compositions are formed into a definite shaped article, such as by casting. While we do not wish to be bound by any explanation of the photochromic mechanism which results or theory in regard thereto, it is possible that the active material may be formed by the formation of a metal adduct with the polymer. For example, utilizing poly(methyl methacrylate) and tungsten hexachloride, the photochromism could possibly result by formation of a tungsten addition product with a reactive oxygen in the polymer. The same result could also occur when the solvent present, if any, has a reactive oxygen therein.

The scope of the present invention is also of such breadth so as to include the use of such modifying materials as fillers, lubricants, plasticizers, stabilizers, antioxidants and the like as additives to the novel compositions claimed herein in addition to ultraviolet light absorbers.

The novel compositions of the present invention may be used to produce such articles as plastic window panes, sky lights, automobile windshields, sunglass lenses, memory devices such as optical analogue computers, temporary oscilloscopes, temporary photographic proofs, photographic marking devices, light switches, optical masks, wall panels, jewelry, toys, advertising articles and the like.

The following examples are set forth for purposes of illustration only and are not to be construed as limitations on the instant invention except as set forth in the appended claims. All parts and percentages are by weight unless otherwise specified.

#### EXAMPLE I

A composition of matter is produced by blending 20 parts of polymethylmethacrylate, dissolved in 80 parts of dioxane, with 2.5 parts of tungsten hexachloride. To this composition of matter are then added 0.25 mol of  $\text{FeCl}_3$  per mole of tungsten hexachloride. The resultant solution is stirred, filtered and then cast as a film, 20 mils in thickness, on a sheet of commercially available polyethyleneglycol terephthalate. The film is dried and, when irradiated with ultraviolet light, changes from colorless to blue. The bleaching (optical density) of the film from blue to colorless is then measured in a spectrophotometer after 30 minutes in the dark and at room temperature. The results of Example 1 and of additional metal salt additives, solvents, polymers and transition metals are set forth in Table I below.

TABLE I

| Ex. | Metal Salt Additive                   | Oxidation Potential | Mols <sup>1</sup> Additive | Polymer                                    | Transition Metal Compound                                                       | Solvent             | Percent <sup>2</sup> Bleached | P.C. |
|-----|---------------------------------------|---------------------|----------------------------|--------------------------------------------|---------------------------------------------------------------------------------|---------------------|-------------------------------|------|
| 1   | FeCl <sub>3</sub>                     | -0.77               | 0.25                       | PMMA                                       | WCl <sub>3</sub>                                                                | Dioxane             | 0.60                          | Yes. |
| 2   |                                       |                     |                            | PMMA                                       | WCl <sub>3</sub>                                                                | do                  | 0.72                          | Yes. |
| 3   | Na <sub>2</sub> HASO <sub>4</sub>     | -0.56               | 0.25                       | PMMA                                       | WCl <sub>6</sub>                                                                | do                  | 0.51                          | Yes. |
| 4   | TiCl <sub>3</sub>                     | -1.24               | 0.25                       | PMMA                                       | WCl <sub>6</sub>                                                                | do                  | 0.61                          | Yes. |
| 5   | MnCl <sub>2</sub>                     | -1.51               | 0.25                       | PMMA                                       | WCl <sub>6</sub>                                                                | Dioxane             | 0.45                          | Yes. |
| 6   | Mn(O-C-CH <sub>3</sub> ) <sub>2</sub> | -1.51               | 0.10                       | Polystryrene                               | WOCl <sub>4</sub>                                                               | Glyne               | 0.47                          | Yes. |
| 7   | Ce(SO <sub>4</sub> ) <sub>2</sub>     | -1.61               | 0.50                       | Thermoplastic polyester resin <sup>3</sup> | NbCl <sub>5</sub>                                                               | Dimethyl sulfoxide  | 0.50                          | Yes. |
| 8   | TiCl <sub>3</sub>                     | -1.25               | 0.20                       | Cellulose acetate                          | Ti(OCH <sub>3</sub> ) <sub>4</sub>                                              | Acetone             | 0.58                          | Yes. |
| 9   | RhCl <sub>3</sub>                     | -1.46               | 0.10                       | Polyurethane resin <sup>4</sup>            | CrO <sub>2</sub> Cl <sub>2</sub>                                                | Dimethyl formamide  | 0.51                          | Yes. |
| 10  | K <sub>3</sub> IrCl <sub>6</sub>      | -1.02               | 0.20                       | Poly(acrylic acid)                         | NbO <sub>3</sub>                                                                | Ethylene glycol     | 0.45                          | Yes. |
| 11  | MnCl <sub>2</sub>                     | -1.51               | 0.15                       | Poly(vinylacetate)                         | WO <sub>2</sub> (O <sub>2</sub> H <sub>5</sub> ) <sub>2</sub>                   | None                | 0.49                          | Yes. |
| 12  | FeCl <sub>3</sub>                     | -0.77               | 0.10                       | Poly(acrylic acid)                         | ZrCl <sub>4</sub>                                                               | Methylethyl ketone  | 0.58                          | Yes. |
| 13  | TiCl <sub>3</sub>                     | -1.25               | 0.15                       | Poly(oxymethylene)                         | TaCl <sub>5</sub>                                                               | None                | 0.58                          | Yes. |
| 14  | TiCl <sub>3</sub>                     | -1.25               | 0.50                       | Poly(methylacrylate)                       | WBr <sub>6</sub>                                                                | Dioxane             | 0.55                          | Yes. |
| 15  | Mn(O-C-CH <sub>3</sub> ) <sub>2</sub> | -1.51               | 0.10                       | Cellulose acetate butyrate                 | TiOF <sub>2</sub>                                                               | Gamma-valerolactone | 0.52                          | Yes. |
| 16  | Na <sub>2</sub> HASO <sub>4</sub>     | -0.56               | 0.05                       | Poly(vinylbutyral)                         | HfCl <sub>4</sub>                                                               | Acetic acid         | 0.50                          | Yes. |
| 17  | MnCl <sub>2</sub>                     | -1.51               | 0.10                       | Poly(acetaldehyde)                         | WF <sub>6</sub>                                                                 | Acetone             | 0.46                          | Yes. |
| 18  | AgCl <sub>2</sub>                     | -1.98               | 0.20                       | PMMA                                       | WCl <sub>3</sub>                                                                | Dioxane             | 0.73                          | Yes. |
| 19  | GeCl <sub>4</sub>                     | +0.52               | 0.15                       | PMMA                                       | WCl <sub>3</sub>                                                                | do                  | 0.72                          | Yes. |
| 20  | FeCl <sub>2</sub>                     | -0.77               | 0.25                       | Polyacrylonitrile                          | VO(O <sub>2</sub> C <sub>2</sub> H <sub>5</sub> ) <sub>3</sub>                  | Dimethyl formamide  | 0.61                          | Yes. |
| 21  | TiCl <sub>3</sub>                     | -1.25               | 0.10                       | Polyamide resin <sup>5</sup>               | ZrBr <sub>2</sub> (OC <sub>2</sub> H <sub>5</sub> ) <sub>2</sub>                | Benzyl alcohol      | 0.59                          | Yes. |
| 22  | K <sub>3</sub> IrCl <sub>6</sub>      | -1.02               | 0.15                       | Polyvinylchloride                          | TaOl <sub>3</sub>                                                               | None                | 0.00                          | No.  |
| 23  | MnCl <sub>2</sub>                     | -1.51               | 0.30                       | Terpolymer MMA/ST/AN 60/20/20              | W <sub>2</sub> I <sub>2</sub> (OC-C <sub>10</sub> H <sub>6</sub> ) <sub>4</sub> | Methylethyl ketone  | 0.48                          | Yes. |
| 24  | NaHASO <sub>4</sub>                   | -0.56               | 0.20                       | Polycarbonate resin <sup>6</sup>           | TiCl <sub>4</sub>                                                               | Ethylene dichloride | 0.56                          | Yes. |

<sup>1</sup> Per mol of transition metal compound.<sup>2</sup> Optical density of sample measured in spectrophotometer after 30 minutes in the dark at room temperature. 1.00 indicates no bleaching and 0.00 indicates complete bleaching.<sup>3</sup> Commercially available polyester resin produced from 50% phthalic acid, 25% diethylene glycol and 25% dipropylene glycol.<sup>4</sup> Commercially available polyurethane resin produced by reacting a polyester resin of diethylene glycol, hexanediol-1,3 and phthalic acid with 2,4-toluenediisocyanate.<sup>5</sup> Commercially available polyamide resin produced from hexamethylene diamine and adipic acid.

I claim:

1. A composition of matter comprising (1) a polymer, (2) a solvent therefor, (3) a metal compound having the formula



wherein M is a metal selected from the group consisting of titanium, zirconium, tungsten, hafnium, tantalum, zirconium, chromium, vanadium and niobium, X is a halide, R is selected from the group consisting of an alkyl radical having from 1-12 atoms, inclusive, an aryl radical having from 6-10 carbon atoms, inclusive, and

R<sup>1</sup> is selected from the group consisting of an alkyl radical having from 1-12 carbon atoms inclusive, and an aryl radical having from 6-10 carbon atoms, inclusive, m and p are whole positive integers of from 0-6 inclusive, and n is a whole positive integer of from 0-2, inclusive, the total of 2n plus m plus p being equal to the valence of the metal M, at least 1 of m and p being an integer of at least 1, at least one of said polymer and said solvent containing oxygen, and (4) 0.01 mol to 5.0 mols, per mol of (2), of a metal salt which, in solution, has an oxidation potential of from about -30 to about -1.65.

2. A composition according to claim 1 wherein said polymer is poly(methylmethacrylate).

3. A composition according to claim 1 wherein said metal compound is tungsten hexachloride.

4. A composition according to claim 1 wherein said solvent is dioxane.

5. A composition according to claim 1 wherein said polymer is poly(methylmethacrylate), said solvent is dioxane and said metal compound is tungsten hexachloride.

6. A composition of matter according to claim 1 wherein said polymer is poly(methylmethacrylate), said metal

<sup>6</sup> Commercially available carbonate resin produced from reacting phosgene with bisphenol A to give product having a structure

CODE.—PMMA K Poly(methyl methacrylate), MMA K Methyl methacrylate, ST K Styrene, AN K Acrylonitrile, P.C. K photochromic compound is niobium pentachloride and said solvent is ethyl acetate.

7. A composition according to claim 1 wherein the metal salt is thallous chloride.

8. A composition according to claim 1 wherein the metal salt is manganese chloride.

9. A composition of matter comprising (1) an oxygen-containing polymer, (2) a metal compound having the formula



wherein M is a metal selected from the group consisting of titanium, zirconium, tungsten, hafnium, tantalum, zirconium, chromium, vanadium and niobium, X is a halide, R is selected from the group consisting of an alkyl radical having from 1-12 atoms, inclusive, an aryl radical having from 6-10 carbon atoms, inclusive, and

R<sup>1</sup> is selected from the group consisting of an alkyl radical having from 1-12 carbon atoms, inclusive, and an aryl radical having from 6-10 carbon atoms, inclusive, m and p are whole positive integers of from 0-6 inclusive, and n is a whole positive integer of from 0-2, inclusive, the total of 2n plus m plus p being equal to the valence of the metal M, at least 1 of m and p being an integer of at least 1 and (3) 0.01 mol to 5.0 mols per mol of (2), of a metal salt which, in solution, has an oxidation potential of from about -30 to about -1.65.

10. A composition according to claim 9 wherein said polymer is poly(methylmethacrylate).

11. A composition according to claim 9 wherein said metal compound is tungsten hexachloride.

12. A composition according to claim 9 wherein said polymer is poly(methylmethacrylate) and said metal compound is niobium pentachloride.

13. A composition according to claim 9 wherein the metal salt is manganese chloride.

13

14. A composition according to claim 9 wherein the metal salt is thallous chloride.

**References Cited**

Brown, G. H.: Phototropy, A Literature Review, December 1959, AD #234,009, pp. 18-20, 96-90 PC.  
El-Sayed, "New Class of Photochromic Substances:

14

"Carbonyls," Jr. Phys. Chem., 68, 433-4 (1964), 96-90 PC.

Singh, G.: "Phototropy of Inorganic Salts," J. Chem. Soc., 121, 782-5 (1822), 96-90 PC.

NORMAN G. TORCHIN, *Primary Examiner.*  
C. E. DAVIS, *Assistant Examiner.*